

June 6, 1961

T. A. STERNBERG

2,987,423

HEAT RADIATING COATINGS

Filed Sept. 26, 1958

2 Sheets-Sheet 1

PREPARE FIRST SLURRY COMPRISING AN OXIDE OF IRON OR NICKEL, OR A MIXTURE OF THESE OXIDES, WITH AN ORGANIC BINDER AND A SOLVENT FOR SAID BINDER.

COAT FIRST SLURRY ON A METALLIC BASE, FOR EXAMPLE ON A ROLL OF STRIP CONSISTING OF EITHER IRON, NICKEL, A FERROUS ALLOY, A NICKEL ALLOY, OR A NICKEL-COATED ALLOY.

DRY THE STRIP BY HEATING IT FOR A FEW MINUTES AT 100°-200° C.

REDUCE THE OXIDE TO THE SPONGY METAL BY HEATING THE STRIP IN A REDUCING ATMOSPHERE, FOR EXAMPLE IN FORMING GAS.

SINTER THE SPONGY METAL TO THE STRIP.

PREPARE SECOND SLURRY COMPRISING COMMINUTED ALUMINUM, AN ORGANIC BINDER, AND A SOLVENT FOR SAID BINDER, E.G., AN ESTER.

APPLY SECOND SLURRY OVER THE SINTERED SURFACE ON THE STRIP.

DRY THE STRIP BY HEATING FOR A FEW MINUTES AT 100°-200° C.

FORM THE STRIP INTO PARTS SUCH AS ELECTRON TUBE COMPONENTS.

HEAT THE PARTS IN HYDROGEN FURNACE AT ABOUT 600° C. FOR A FEW MINUTES TO REDUCE THE ORGANIC BINDER.

FIRE THE FORMED PARTS IN VACUUM AT ABOUT 725°-1000° C. TO PRODUCE A ROUGH DARK HEAT-RADIATING SURFACE.

INVENTOR.

THEODORE A. STERNBERG

BY

W.S. Hill

AGENT

Fig. 1.

June 6, 1961

T. A. STERNBERG

2,987,423

HEAT RADIATING COATINGS

Filed Sept. 26, 1958

2 Sheets-Sheet 2

Fig. 2.



INVENTOR.

THEODORE A. STERNBERG

BY

*W.S. Hill*

AGENT

## 1

2,987,423

## HEAT RADIATING COATINGS

Theodore A. Sternberg, Basking Ridge, N.J., assignor to  
Radio Corporation of America, a corporation of Delaware.

Filed Sept. 26, 1958, Ser. No. 763,704  
14 Claims. (Cl. 117—217)

This invention relates to a method of coating metal articles to improve their ability to radiate heat. The process of the instant invention is particularly applicable to the manufacture of coated iron or nickel parts for use in vacuum tubes and the like.

Electron tubes and the like are usually provided with a cathode having a coated surface which readily emits electrons, and an anode which collects the emitted electrons. The anode is bombarded by electrons during the operation of the tube, and therefore heats up rapidly. This heat must be dissipated before the temperature of the tube becomes too high for efficient operation, due to gas evolution or reverse emission. Since convection and conduction processes cannot be utilized to remove heat in these applications, it is necessary that the anode surface be a good heat radiator. Tube components such as anodes are therefore treated to provide rough dark surfaces, which are known to be more efficient heat radiators than smooth bright surfaces.

One method of obtaining an efficient heat-radiating surface is to coat the metallic anode with aluminum, thus obtaining a smooth bright surface, and subsequently heat treating the anode to convert the bright surface, which is a poor heat radiator into a rough dark surface which is an efficient heat radiator. The converting of a smooth bright surface into a rough dark surface is known in the vacuum tube art as alitizing.

Vacuum tube parts such as anodes are commonly made of ferrous or nickel alloys. Nickel-coated alloys such as clad steels and nickel-iron alloys are also utilized for this purpose. These base materials are usually supplied as rolls of flexible strip, and have previously been coated with aluminum either by dipping in molten aluminum, or by cladding, for example by cold rolling steel strip between two strips of aluminum. The aluminum coating thus formed is a poor heat radiator, being smooth and bright. The strip is then formed into anodes and various other electron tube parts, such as plates, beam plates and grid collars, and thereafter heat treated to convert the bright aluminum coating into a rough dark surface which is an excellent heat radiator. However, satisfactory aluminum-coated strip is relatively expensive, since the dip process, which is similar to that described in U.S. Patent 2,110,893, is subject to oxidation and requires special ambients. The clad materials require heavy presses and high pressures, and even then the aluminum does not adhere to the strip unless both have been carefully cleaned, pickled, brushed, and sand blasted. Moreover, clad material is not readily available from domestic sources, so that imported aluminum-coated material must be relied upon.

An object of this invention is the provision of an improved method of forming an improved heat-radiating surface on a metallic base.

Another object is the provision of an inexpensive process for forming an efficient heat-reducing surface on a metallic base.

Still another object is the provision of an improved method for making aluminum-coated strip.

Yet another object is the provision of a method of making alitized metal parts from domestic materials.

These and other objects are provided by the instant invention, in which a base material such as metallic strip selected from the group consisting of nickel, iron, ferrous alloys, nickel alloys, and nickel-coated alloys, is coated

## 2

with a first slurry comprising a material selected from the group consisting of iron oxide, nickel oxide, and mixtures of iron and nickel oxides. The first slurry is dried, and the oxide is then reduced to the metal. The spongy reduced metal is thereafter sintered, and a second slurry comprising comminuted aluminum such as finely divided powder or flakes is applied to the sintered reduced metal. Next the second slurry is dried, leaving an aluminum-coated surface over the base. Last, the base material is alitized by heat treatment in vacuum to produce a rough dark surface which is an efficient heat radiator. The last step is preferably performed after the base material has been formed into an electron tube part and has been inserted in the tube.

15 The invention and its advantages will be described in greater detail with reference to the accompanying drawing, in which:

FIGURE 1 is a flow sheet showing the various steps of the alitizing process;

20 FIGURE 2 is a schematic diagram of one type of apparatus useful in performing the process of this invention.

25 As shown in FIGURE 1, the first step in the process is the preparation of the first slurry, which comprises an oxide of iron or nickel, or a mixture of these oxides. A mixture containing about 1-20% by weight nickel oxide, and the balance iron oxide, has been found particularly suitable. Any of the three oxides of iron ( $FeO$ ,  $Fe_2O_3$ ,  $Fe_3O_4$ ) and the two oxides of nickel ( $NiO$ ,  $Ni_2O_3$ ) may be utilized. The powdered oxide is mixed with an organic binder, such as nitrocellulose or carboxymethylcellulose or the like, and an organic solvent which is capable of dissolving the binder. The proportions of these ingredients are adjusted so that the slurry contains from 10-80% by weight of the oxides. At higher concentrations, the slurry becomes an extremely thick paste. A concentration of about 20% by weight of the oxide in the slurry has been found suitable for many applications.

30 The method may be best understood with reference to a particular example. In this example, a mixture of 99% ferric oxide  $Fe_2O_3$  and 1% nickel oxide  $NiO$  (by weight) is used to make the first slurry. Ten pounds of the mixed oxides which have been powdered to pass 150-375 mesh are ball milled for about 3 hours with 1220 cc. 35 of an organic solvent such as an ester or a ketone. In this example, the solvent is butyl acetate. A 4 gallon mill containing 28 pounds of three-quarter inch steel balls is utilized. The powder has a consistency (North Standard) of 4.0 before the mixing, and 6.0 (semi-paste) after mixing. Another 550 cc. of butyl acetate is added, and milling is continued for about 2 hours until the mixture reaches a pasty consistency (North Standard 6.75). Now 190 cc. of butyl acetate and 1610 cc. of nitrocellulose (40 sec cotton) is added, and the mixture is ball milled to a paint-like consistency.

40 The first slurry is then applied to the base, which may be nickel, iron, nickel alloys, ferrous alloys such as steel, or nickel clad steels. In this example, the base consists of steel strip about 7 inches wide and about 5 mils thick. These dimensions are not critical, and the strip may for example be 4 to 10 mils thick. The apparatus shown in FIGURE 2 may be utilized to perform the process in a continuous manner, the strip being spooled through the apparatus at about 2 to 7 feet per minute. The speed is adjusted in accordance with the apparatus dimensions, and the temperatures of the driers and ovens. In this example, the strip 10 travels at the rate of 5 feet per minute from roll 11 into applicator 12, where it receives, 45 a coating of the first slurry 13. The coating is about the thickness and consistency of paint.

50 The coated strip is then dried in air. Since drying at room temperature is too slow, the strip 10 is passed

through a drier 14 which is maintained at about 100-200° C. In this example, the temperature of the drier is kept at about 160° C. A dried layer of the mixed iron oxide and nickel oxide is left on the surface of the strip.

The next step in the process is the reduction of the oxide coating to the metal by heating the strip in a reducing atmosphere at a temperature of about 800 to 1000° C. The residue of the organic binder is reduced and volatilized during this step. In this example, the strip 10 is passed through a hydrogen furnace 15 which contains two sets of heaters 16 and 16'. A thermocouple 17 between the two sets of heaters and about 2 inches away from the strip is used to monitor the furnace temperature. The power supply is regulated so that a temperature of about 975° C. is maintained in the center of the furnace 15. A stream of hydrogen is passed into the furnace at inlet 18 and leaves at outlet 19. The pressure of hydrogen is maintained slightly above atmospheric, in order to exclude air from the furnace. Other reducing ambients such as forming gas may be utilized. As the strip 10 passes through the lower or reduction zone of the furnace, the oxide coating is reduced to the metal.

The reduced metal, whether iron, nickel, or a mixture of these, is rough and spongy, but does not adhere well to the strip. For this reason the spongy metal is sintered by heating the strip at a temperature below the melting point of the strip and the spongy metal layer. A second furnace is not required, since this step may be performed under the same conditions as the previous reduction step. The strip 10 passes between the second set of heaters 16' in the furnace 15, and is thereby heated sufficiently to sinter the spongy metal and improve its adherence to the strip.

The strip 10 is next rolled through applicator 20, where it is coated with the second slurry 21, which comprises comminuted or finely divided aluminum together with an organic binder and a solvent for the binder. The aluminum may be in the form of a powder or flakes, and the concentration of the aluminum in this slurry may vary from about 5% to 20% by weight. In this example, the second slurry 21 is prepared by mechanically mixing or ball milling 5 pounds of flake aluminum with 4530 cc. of nitrocellulose (40 sec cotton) as binder and 13,590 cc. of butyl acetate as solvent. This mixture contains about 10% by weight aluminum, although slurries with about 5% to 20% by weight aluminum may also be utilized. The second slurry 21 adheres to the sintered metal surface on the strip 10, and forms a coating about .1 to .5 mil thick.

The strip is again dried in air. Since drying at room temperature is too slow, the strip 10 is passed through a second drier 22, which is maintained at 100-200° C. In this example, the drier 22 is kept at about 160° C.

The strip may then be rolled and stored, or sent directly to a slitting machine where it is cut into portions of appropriate size. The portions are then formed into the desired parts, for example electron tube components such as anodes, beam plates, and grid collars.

For vacuum tube applications, it is desirable to reduce the residue of the organic binder on the surface of the parts so as to prevent the subsequent evolution of gases when the parts are used as vacuum tube components. Reduction may be accomplished by heating the parts in a reducing ambient for a few minutes at a temperature high enough to insure rapid reduction of the binder. In this example, the parts are heated in a hydrogen furnace for about 2-3 minutes at about 600° C. This heating cycle is not sufficient to alitize the aluminum-coated surfaces of the parts, which remain smooth and bright.

The last step is the alitzing of the parts by heating them in vacuum at about 725-1000° C. In this example, the parts are anodes, which are inserted into glass tubes.

While the tubes are being evacuated, the tube components are heated to about 725-1000° C. In this example, the anodes are heated to about 850° C. during the alitzing step. The surface of the anode changes color during this step from smooth shiny bright, which is a poor heat radiator, to a rough dark slate gray, which is an efficient heat radiator.

There has thus been described an improved method of providing an efficient heat-radiating surface on metal parts such as vacuum tube anodes. The method is not limited to electron tube components, and may be applied wherever a good heat-radiating surface is required. It will be understood that various modifications may be made in the process without departing from the spirit and scope of the instant invention. For example, the slurries may be made with other binders such as potato starch and corn starch, and with other solvents such as ethyl acetate and propyl acetate.

What is claimed is:

20. 1. A method of providing a heat-radiating surface on a base selected from the group consisting of nickel, iron, ferrous alloys, nickel alloys, and nickel-coated alloys, which comprises coating said base with a first slurry comprising a material selected from the group consisting of iron oxide, nickel oxide, and mixtures of iron and nickel oxides, drying said first slurry, reducing said oxide to the metal, sintering said metal to said base, applying to said sintered metal a second slurry comprising comminuted aluminum, drying said second slurry, and subsequently heating in vacuum to produce a heat-radiating surface.
25. 2. A method of providing a heat-radiating surface on steel strip, which comprises coating said strip with a first slurry comprising a material selected from the group consisting of iron oxide, nickel oxide, and mixtures of iron and nickel oxides, drying said first slurry, reducing said oxide to the metal, sintering said metal to said strip, applying to said sintered metal a second slurry comprising comminuted aluminum, drying said second slurry, and subsequently heating said strip in vacuum to produce a heat-radiating surface on said strip.
30. 3. A method of providing a heat-radiating surface on steel strip, which comprises coating said strip with a first slurry comprising iron oxide, heating said strip to dry said first slurry, reducing said oxide to iron, sintering said iron to said strip, applying to said sintered iron a second slurry comprising comminuted aluminum, heating said strip to dry said second slurry, and subsequently heating said strip in vacuum to produce a heat-radiating surface on said strip.
35. 4. A method of providing a heat-radiating surface on a base selected from the group consisting of nickel, iron, ferrous alloys, nickel alloys, and nickel-coated alloys, which comprises coating said base with a first slurry comprising iron oxide and nickel oxide, the weight of the nickel oxide being 1-20% of the weight of the iron oxide, heating said base to dry said first slurry, reducing said oxides to the metal, sintering said metal to said base, applying to said sintered metal a second slurry comprising comminuted aluminum, heating said base to dry said second slurry, and subsequently heating said base in vacuum to produce a heat-radiating surface on said base.
40. 5. A method of providing a heat-radiating surface on a base selected from the group consisting of nickel, iron, ferrous alloys, nickel alloys, and nickel-coated alloys, which comprises coating said base with a first slurry comprising an organic binder, a solvent for said binder, and a material selected from the group consisting of iron oxide, nickel oxide, and mixtures of iron and nickel oxides, heating said base to dry said first slurry, reducing said oxide to the metal, sintering said metal to said base, applying to said sintered metal a second slurry comprising an organic binder, a solvent for said binder, and

commminuted aluminum, heating said base to dry said second slurry, and subsequently heating said base in vacuum to produce a heat-radiating surface on said base.

6. A method of providing a heat-radiating surface on a base selected from the group consisting of nickel, iron, ferrous alloys, nickel alloys, and nickel-coated alloys, which comprises coating said base with a first slurry comprising an organic binder, a solvent for said binder, and a material selected from the group consisting of iron oxide, nickel oxide, and mixtures of iron and nickel oxides, said slurry containing 10% to 80% by weight of said oxide, heating said base to dry said first slurry, reducing said oxide to the metal, sintering said metal to said base, applying to said sintered metal a second slurry comprising an organic binder, a solvent for said binder, and comminuted aluminum, said aluminum powder comprising 5% to 20% by weight of said second slurry, heating said base to dry said second slurry, and subsequently heating said base in vacuum to produce a rough dark heat-radiating surface on said base.

7. A method of providing a heat-radiating surface on a base selected from the group consisting of nickel, iron, ferrous alloys, nickel alloys, and nickel-coated alloys, which comprises coating said base with a first slurry comprising an organic binder, a solvent for said binder, and a material selected from the group consisting of iron oxide, nickel oxide, and mixtures of iron and nickel oxides, said slurry containing about 20% by weight of said oxide, heating said base to dry said first slurry, reducing said oxide to the metal, sintering said metal to said base, applying to said sintered metal a second slurry comprising an organic binder, a solvent for said binder, and aluminum powder, said comminuted aluminum comprising about 10% by weight of said second slurry, heating said base to dry said second slurry, and subsequently heating said base in vacuum to produce a rough dark heat-radiating surface on said base.

8. A method of providing a heat-radiating surface on a base selected from the group consisting of nickel, iron, ferrous alloys, nickel alloys, and nickel-coated alloys, which comprises coating said base with a first slurry comprising an organic binder, a solvent for said binder, and a material selected from the group consisting of iron oxide, nickel oxide, and mixtures of iron and nickel oxides, heating said base at a temperature of 100 to 200° C. to dry said first slurry, reducing said oxide to the metal, sintering said metal to said base, applying to said sintered metal a second slurry comprising an organic binder, a solvent for said binder, and comminuted aluminum, heating said base at a temperature of 100 to 200° C. to dry said second slurry, and subsequently heating said base in vacuum to produce an alitized aluminum-coated surface on said base.

9. A method of providing a heat-radiating surface on steel strip, which comprises coating said strip with a first slurry comprising iron oxide, heating said strip at about 160° C. to dry said first slurry, reducing said oxide to iron, sintering said iron to said strip, applying to said sintered iron a second slurry comprising comminuted aluminum, heating said strip to about 160° C. to dry said second slurry, and subsequently heating said strip in vacuum to produce an alitized aluminum-coated surface on said strip.

10. A method of providing a heat-radiating surface on steel strip, which comprises coating said strip with a first slurry comprising iron oxide, heating said strip at about 160° C. to dry said first slurry, reducing said oxide to iron, sintering said iron to said strip, applying to said sintered iron a second slurry comprising comminuted aluminum, heating said strip to about 160° C. to dry said second slurry, and subsequently heating said strip in vacuum at a temperature about 725-1000° C. to produce an alitized aluminum-coated surface on said strip.

11. A method of providing a heat-radiating surface on steel strip, which comprises coating said strip with a first slurry comprising iron oxide, heating said strip at about 160° C. to dry said first slurry, heating said base in a reducing atmosphere at a temperature of 800-1000° C. so as to reduce said oxide to iron, sintering said iron to said strip, applying to said sintered iron a second slurry comprising comminuted aluminum, heating said strip to about 160° C. to dry said second slurry, and subsequently heating said strip in vacuum at a temperature of about 725-1000° C. to produce an alitized aluminum-coated surface on said strip.

12. A method of providing a heat-radiating surface on steel strip, which comprises coating said strip with a first slurry comprising iron oxide, heating said strip at about 160° C. to dry said first slurry, heating said base in a hydrogen atmosphere at 975° C. so as to reduce said oxide to iron, sintering said iron to said strip, applying to said sintered iron a second slurry comprising comminuted aluminum, heating said strip to about 160° C. to dry said second slurry, and subsequently heating said strip in vacuum at a temperature of about 725-1000° C. to produce an alitized aluminum-coated surface on said strip.

13. A method of providing a heat-radiating surface on a base selected from the group consisting of nickel, iron, ferrous alloys, nickel alloys, and nickel-coated alloys, which comprises coating said base with a first slurry comprising an organic binder, a solvent for said binder, and a material selected from the group consisting of iron oxide, nickel oxide, and mixtures of iron and nickel oxides, said slurry containing 10% to 80% by weight of said oxide, heating said base at a temperature of 100-200° C. to dry said first slurry, reducing said oxide to the metal, sintering said metal to said base, applying to said sintered metal a second slurry comprising an organic binder, a solvent for said binder, and comminuted aluminum, said aluminum comprising 5% to 20% by weight of said slurry, heating said base at a temperature of 100-200° C. to dry said second slurry, and subsequently heating said base in vacuum to produce an alitized aluminum-coated surface on said base.

14. A method of providing a heat-radiating surface on a base selected from the group consisting of nickel, iron, ferrous alloys, nickel alloys, and nickel-coated alloys, which comprises coating said base with a first slurry comprising an organic binder, a solvent for said binder, and a material selected from the group consisting of iron oxide, nickel oxide, and mixtures of iron and nickel oxides, said slurry containing 10% to 80% by weight of said oxide, heating said base at a temperature of 100-200° C. to dry said first slurry, heating said base in a reducing atmosphere at a temperature of 800-1000° C. so as to reduce said oxide to the metal, sintering said metal to said base, applying to said sintered metal a second slurry comprising an organic binder, a solvent for said binder, and comminuted aluminum, said aluminum comprising 5% to 20% by weight of said second slurry, heating said base in air at a temperature of 100-200° C. to dry said second slurry, firing said base in hydrogen to reduce said organic binder, and subsequently heating said base in vacuum to produce an alitized aluminum-coated surface on said base.

References Cited in the file of this patent

UNITED STATES PATENTS

|           |               |               |
|-----------|---------------|---------------|
| 2,197,622 | Sendzimir     | Apr. 16, 1940 |
| 2,300,400 | Axline        | Nov. 3, 1942  |
| 2,328,788 | Deputy        | Sept. 7, 1943 |
| 2,539,246 | Hensel        | Jan. 23, 1951 |
| 2,541,813 | Frisch et al. | Feb. 13, 1951 |
| 2,744,838 | Newman        | May 8, 1956   |
| 2,840,493 | Okress        | June 24, 1958 |